

## UNITED STATES PATENT OFFICE

1,972,588

## FROTH-FLOTATION PROCESS

Mahlin S. Hansen, Indianapolis, Ind., assignor to  
 Peter C. Reilly, Indianapolis, Ind.

No Drawing. Application August 19, 1932,  
 Serial No. 629,423

10 Claims. (Cl. 209—166)

This invention relates to improvements in the concentration of minerals of "oxidized ores" by the froth-flotation process. More particularly, the invention aims to improve the efficiency of 5 the froth-flotation process as applied to "oxidized ores", by the use of certain modifying agents which have the double effect of activating the desired "oxidized minerals" so that they are made more amenable to froth-flotation and of dis-  
 10 persing slimes.

Certain minerals have not heretofore been readily amenable to the froth-flotation process, and have required relatively large quantities of 15 the selector reagents to effect their flotation. An important class of these is the "oxidized minerals" which are present in "oxidized ores"; and it is to these that my present invention is directed. By "oxidized ores" I mean those ores which are 20 commonly so known to miners and millmen; and which may be partly or wholly true carbonates, but are often partly or largely sulfates, hydrox-ides, oxides, and analogous compounds, and are 25 usually quite complex. Among the minerals which may be included in the term "oxidized min-  
 30 erals" may be mentioned phosphate rock, fluo-rspar, phosphate, talc, barite, calcite, feldspar, garnet, hematite, manganese-calcite, malachite, pyrolusite, rhodochrosite, scheelite, and wolfram-ite. Because of the relatively low unit value of 35 the minerals of this group, and because of the relatively high quantity of selector reagents heretofore necessary to effect flotation, the application of the froth-flotation process to their con-centration has been in general uneconomical.

35 Further, with most ores, including those containing oxidized minerals, the presence of slimes in the pulp has been a serious impediment to the successful concentration of the mineral values by the froth-flotation process, and in many cases 40 the presence of slimes has in itself prevented the concentration of mineral even when the mineral was otherwise readily amenable to flotation.

This invention is based upon the discovery that 45 in the application of the froth-flotation process to the flotation of "oxidized-minerals" in "oxi-dized ore" pulps, the use in regulated small quan-tities of a fluosilicate of the class including cop-  
 50 per fluosilicate (such as  $CuSiF_6 \cdot 6H_2O$ ), silver fluosilicate (such as  $Ag_2SiF_6 \cdot 4H_2O$ ), zinc fluo-silicate (such as  $ZnSiF_6 \cdot 6H_2O$ ), cadmium fluo-silicate (such as  $CdSiF_6 \cdot 6H_2O$ ), mercury fluo-silicate (such as  $HgSiF_6 \cdot H_2O$ ), and lead fluo-silicate (such as  $PbSiF_6 \cdot 6H_2O$  and  $PbSiF_6 \cdot 4H_2O$ ), markedly aids in effecting selection of valuable mineral from gangue. The use of one or more of

these fluosilicate compounds makes it possible to apply the froth-flotation process in the con-centration of "oxidized minerals" at greatly re-duced cost, and in some cases where it has not heretofore been commercially practical. 60

The following advantages are obtained by the use of the aforesaid modifying agents:

(1) A decrease is made in the amount of selec-tor reagents required to effect flotation. 65

(2) A dispersion of slime from both the min-eral surfaces and the froth surfaces is accom-plished; which obviates the deleterious effect of slimes. 70

(3) In general, a more brittle froth is obtained, which permits greater selectivity in the differen-tial or preferential flotation of minerals. 75

One hypothesis as to the activating action in the flotation circuit by the fluosilicates of metals of the class comprising copper, silver, zinc, cad-mium, mercury, and lead, is as follows: 80

The cations of these salts in solution exchange for cations on the mineral surface, thereby pro-  
 85 ducing a surface which is more amenable to the froth-flotation process and more readily affected by selector flotation reagents. In addition to this cation effect, the slimes-dispersion which I ob-tain both from the mineral surfaces and from the froth surfaces is due to the highly effective action of the anions of such fluosilicates in solu-tion. The slime-freed mineral surfaces are clean 90 and unobstructed surfaces for the action of the selector flotation reagents, which makes for greater efficiency and economy. The effect of free-ing the froth of slimes is to provide clean, un-loaded froth surfaces for buoying the mineral 95 particles to be floated.

Examples of the use of these fluosilicates are 95 given below. Example I shows the use of lead fluosilicate and of zinc fluosilicate in the flota-tion of an "oxidized" copper mineral in an ore 100 pulp containing both sands and slimes, in an acid circuit. Example II shows the use of lead fluo-silicate and of cupric fluosilicate in the flotation of the non-metallic mineral feldspar, in an ore pulp substantially free from slimes, in a neutral circuit. Example III shows the use of zinc fluo-silicate in the flotation of an "oxidized" lead min-eral, in an ore pulp containing both sands and slimes, in an alkaline circuit. In these examples 105 the flotation reagents used in conjunction with the fluosilicates are given merely by way of exam-  
 ple, since any suitable flotation reagents (com-prising both froth and selector reagents) may be 110 employed.

*Example I*

The following tests were made on a so-called "oxidized ore" of copper, in which the principal copper mineral was malachite. The ore was ground (minus 100 plus 320 mesh), and fifty-gram charges were used in a Gates-Jacobsen flotation cell with amounts of suitable frother and selector reagents, such as pine oil and butyl dithio-phospho-oleic acid, equivalent to 0.20 lb. and 0.50 lb. respectively per ton of ore, together with activator reagents as shown below in amounts equivalent to pounds per ton of ore as indicated. The hydrogen ion value of the pulp was maintained at pH 6.6.

*Data of Example I*

| Test   | PbSiF <sub>6</sub> .6H <sub>2</sub> O<br>lbs. per ton | ZnSiF <sub>6</sub> .6H <sub>2</sub> O<br>lbs. per ton | Percent re-<br>covery of<br>copper |
|--------|-------------------------------------------------------|-------------------------------------------------------|------------------------------------|
| A..... | None.                                                 | None.                                                 | 0.0                                |
| B..... | 0.25                                                  | None.                                                 | 42.0                               |
| C..... | 0.50                                                  | None.                                                 | 65.0                               |
| D..... | None.                                                 | 0.25                                                  | 50.0                               |
| E..... | None.                                                 | 0.50                                                  | 78.0                               |

*Example II*

The following tests were run on pure orthoclase feldspar mineral (minus 100 plus 320 mesh) using fifty-gram charges in a Gates-Jacobsen flotation cell with amounts of suitable frother and selector reagents, such as pine oil and amyl dithio-phospho-oleic acid, equivalent to 0.20 lb. and 0.75 lb. respectively per ton of mineral, together with such quantities of fluosilicates as activating reagents as are shown below, in quantities equivalent to pounds per ton of mineral as indicated. The hydrogen ion value of the pulp was maintained at pH 7.0.

*Data of Example II*

| Test   | PbSiF <sub>6</sub> .6H <sub>2</sub> O<br>lbs. per ton | CuSiF <sub>6</sub> .6H <sub>2</sub> O<br>lbs. per ton | Percent re-<br>covery of<br>mineral |
|--------|-------------------------------------------------------|-------------------------------------------------------|-------------------------------------|
| F..... | None.                                                 | None.                                                 | 0.0                                 |
| G..... | 1.0                                                   | None.                                                 | 20.0                                |
| H..... | 1.5                                                   | None.                                                 | 31.0                                |
| I..... | None.                                                 | 1.0                                                   | 78.0                                |
| J..... | None.                                                 | 1.5                                                   | 88.0                                |

*Example III*

The following tests were made on an "oxidized" ore of lead. The important characteristics of the ore were as follows:

(1) The ore was high-grade, containing a relatively large amount of lead associated with silver, zinc, and iron;

(2) All of the silver was associated with the lead minerals;

(3) Crushing to 120-mesh was necessary to entirely unlock the economic minerals;

(4) The gangue was decomposed, giving rise to much clay, and contained a large proportion of limestone;

(5) Soluble salts were present which had a marked coagulating effect;

(6) 36% of the lead was present as "oxidized" lead minerals.

The ore was crushed dry to 28-mesh by jaw crushers, followed by wet grinding in a porcelain ball-mill with flint pebbles, to 120-mesh. This product was run over a 12 by 30 inch Wilfley gravity concentrating table, obtaining a relatively coarse lead concentrate containing 20.44%

of the lead content of the ore. The table tailing comprising the oxidized portion of the ore was thickened to a pulp dilution of 4 to 1, and was used for feed in the flotation tests of the following table.

The flotation tests were made with a 500-gram Janney flotation testing machine.

Amounts of suitable sulfidizer, frother, and selector reagents, such as sodium sulfide, pine oil, and sodium xanthate, equivalent to 4.5 lbs., 0.20 lb., and 0.35 lb. respectively per ton of ore,

were added in the order named; together with zinc fluosilicate as an activator reagent, added in order between the sulfidizer and the frother, in amounts equivalent to pounds per ton of ore as indicated. In the flotation feed, the assay was

12.0% lead, 3.0% zinc and 10.8% iron. The hydrogen ion concentration of the pulp circuit was pH 8.4.

*Data of Example III*

| Test   | ZnSiF <sub>6</sub> .6H <sub>2</sub> O<br>lbs. per ton | Assay of concentrate |                       |                  |                       |                  |                       | 100 |  |
|--------|-------------------------------------------------------|----------------------|-----------------------|------------------|-----------------------|------------------|-----------------------|-----|--|
|        |                                                       | Lead                 |                       | Zinc             |                       | Iron             |                       |     |  |
|        |                                                       | Assay<br>Percent     | Recover-<br>y Percent | Assay<br>Percent | Recover-<br>y Percent | Assay<br>Percent | Recover-<br>y Percent |     |  |
| K..... | None.                                                 | 37.5                 | 56.6                  | 3.8              | 14.3                  | 24.0             | 40.7                  | 105 |  |
| L..... | 2.0                                                   | 58.4                 | 81.6                  | 0.6              | 2.0                   | 10.5             | 16.3                  |     |  |

Although I have given specific examples to illustrate my invention, they are illustrative only. Variations in the quantities of reagents employed,

the combinations of reagents, the kinds of "oxidized-ores", the hydrogen ion value of the pulp, and the steps of the procedure, may be varied in practice as determined by the composition of the given "oxidized-ore" without departing from the invention claimed.

For instance, the treatment of the "oxidized-ore" pulp with the fluosilicate or fluosilicates may be by adding the latter to the ore prior to the actual formation of the pulp;

and the term "treating the ore pulp" as used in the claims is intended to include that as well as a treatment after the "oxidized-ore" pulp has been formed.

I have found that the fluosilicates can be used in the crude form as well as in the relatively pure form. The fluosilicate used may be in solid or liquid form, or it may be dissolved in water or other solvent. A plurality of fluosilicates may be used together. I have also found it advantageous at times to form the desired fluosilicate directly in the ore pulp, as for example by the interaction of a fine suspension of cupric hydroxide and a solution of hydrofluosilicic acid, or by a solution of sodium fluosilicate and copper sulphate. Other methods of producing these fluosilicates in the flotation circuit will occur to those skilled in the art.

With some "oxidized ores" it is advantageous to heat the pulp to a temperature of about 90° F. to 130° F.

These fluosilicates can be used with desirable and effective results in alkaline, neutral, or acid circuits. In some cases the action is better in neutral or acid circuits.

I claim as my invention:

1. The process of concentrating "oxidized minerals" from "oxidized ores" by froth flotation, comprising treating an "oxidized-ore" pulp with a fluosilicate of the class consisting of copper fluosilicate, silver fluosilicate, zinc fluosilicate,

- cadmium fluosilicate, mercury fluosilicate, and lead fluosilicate to activate the "oxidized minerals"; and subjecting the treated "oxidized-ore" pulp to the froth-flotation process in the presence 5 of a selector reagent.
2. The process of concentrating "oxidized minerals" from "oxidized ores" by froth flotation, comprising treating an "oxidized-ore" pulp with a fluosilicate of the class consisting of copper fluosilicate, silver fluosilicate, zinc fluosilicate, cadmium fluosilicate, mercury fluosilicate, and lead fluosilicate to activate the "oxidized minerals"; and subjecting the treated "oxidized-ore" pulp to the froth-flotation process in an acid circuit in 10 the presence of a selector reagent.
3. The process of concentrating "oxidized minerals" from "oxidized ores" by froth flotation, comprising treating an "oxidized-ore" pulp with a fluosilicate of the class consisting of copper fluosilicate, silver fluosilicate, zinc fluosilicate, cadmium fluosilicate, mercury fluosilicate, and lead fluosilicate to activate the "oxidized minerals"; and subjecting the treated "oxidized-ore" pulp to the froth-flotation process in a neutral circuit in 15 the presence of a selector reagent.
4. The process of concentrating "oxidized minerals" from "oxidized ores" by froth flotation, comprising treating an "oxidized-ore" pulp with a fluosilicate of the class consisting of copper fluosilicate, silver fluosilicate, zinc fluosilicate, cadmium fluosilicate, mercury fluosilicate, and lead fluosilicate to activate the "oxidized minerals"; and subjecting the treated "oxidized-ore" pulp to the froth-flotation process in an alkaline circuit 20 in the presence of a selector reagent.
5. The process of concentrating "oxidized minerals" from "oxidized ores" by froth flotation, comprising treating an "oxidized-ore" pulp with a fluosilicate of the class consisting of copper fluosilicate, silver fluosilicate, zinc fluosilicate, cadmium fluosilicate, mercury fluosilicate, and lead fluosilicate to activate the "oxidized minerals"; and subjecting the treated "oxidized-ore" pulp to the froth-flotation process in an alkaline circuit 25 in the presence of a selector reagent.
6. The process of concentrating feldspar minerals by froth flotation of pulps of "oxidized ores" containing such feldspar minerals, comprising 80 treating the pulp of such "oxidized ore" with a fluosilicate of the class consisting of copper fluosilicate, silver fluosilicate, zinc fluosilicate, cadmium fluosilicate, mercury fluosilicate, and lead fluosilicate to activate the feldspar minerals; and subjecting such treated "oxidized-ore" pulp to the froth-flotation process in the presence of a selector reagent.
7. The process of concentrating minerals from "oxidized ores" by froth flotation, comprising 85 treating an "oxidized-ore" pulp with copper fluosilicate to activate the "oxidized minerals"; and subjecting the treated "oxidized-ore" pulp to the froth-flotation process in the presence of a selector reagent.
8. The process of concentrating minerals from "oxidized ores" by froth flotation, comprising treating the "oxidized-ore" pulp with zinc fluosilicate to activate the "oxidized minerals"; and subjecting the treated "oxidized-ore" pulp to the froth-flotation process in the presence of a selector reagent.
9. The process of concentrating minerals from "oxidized ores" by froth flotation, comprising 90 treating the "oxidized-ore" pulp with lead fluosilicate to activate the "oxidized minerals"; and subjecting the treated "oxidized-ore" pulp to the froth-flotation process in the presence of a selector reagent.
10. The step in the froth-flotation process of 100 "oxidized-ore" concentration, comprising treating an "oxidized-ore" pulp with a fluosilicate of the class consisting of copper fluosilicate, silver fluosilicate, zinc fluosilicate, cadmium fluosilicate, mercury fluosilicate, and lead fluosilicate to activate the "oxidized minerals", in the presence of a selector reagent.
- MAHLIN S. HANSEN.
- 45 120
- 50 125
- 55 130
- 60 135
- 65 140
- 70 145
- 75 150